

# UNITED STATES PATENT OFFICE.

ATLAS O. CRAIL, OF WARREN, OHIO.

## PROCESS FOR SEASONING WOOD.

1,416,269.

Specification of Letters Patent. Patented May 16, 1922.

No Drawing.

Application filed November 26, 1920. Serial No. 426,498.

To all whom it may concern:

Be it known that I, ATLAS O. CRAIL, a citizen of the United States of America, residing at Warren, in the county of Trumbull and State of Ohio, have invented certain new and useful Improvements in Processes for Seasoning Wood, of which the following is a specification.

This invention relates to the process of 10 seasoning wood by neutralizing the tannic acid therein; expelling it and the water from the pores of the wood, and has for its objects, first, the shrinking of the wood so as to close the pores therein permanently so 15 that further shrinkage by heat or anything else will be impossible; second, to render the process vastly more expeditious and much cheaper.

It is well known that a partial seasoning 20 of wood has been accomplished by keeping it a number of years in a dry atmosphere, and also by first soaking the wood in salted water—ordinarily for perhaps six months, and then drying it in a slow drying kiln at 25 low temperature for some days; and it has been scientifically proven that those processes eliminate but approximately eighty per cent of the moisture and tannic acid as the best known results, so that the wood when 30 made up into furniture or house finishings, can and will because of the warmth of rooms, continue to shrink and produce loose and ill-fitting joints.

My invention saves that time and cures 35 that defect and is completely new, revolutionary and different in fact.

As nearly all wood contains tannic acid and oak contains more than most woods, I cite it as a basis for complete explanation of 40 my invention, applicable to all woods.

The tannic acid I neutralize and eliminate by the use of salt as an alkali, as do others, but in this manner; to-wit—

I fill a covered vat with wood to be seasoned and a five per cent solution of salt and water (about) that is in the proportion of one-half barrel of salt to ten barrels of water.

After the wood, water and salt have been 50 put in the vat and the cover put on, I bring the water to the boiling point and boil it six hours only, (as against six months soaking of other processes).

Meantime I heat a drying kiln up to 250°

F. and at the end of the six hours of boiling 55 remove the wood instantly and immediately the cover of the vat is removed and at once put the wood into the kiln and close the door, where it remains forty-two hours.

The wood is then removed and is reduced 60 to its smallest dimensions, one hundred per cent of the water, salt and tannic acid having been driven out and when jointed and fitted it retains its size and fit indefinitely.

Boiling the wood six hours opens the 65 pores and allows the alkali to combine with the tannic acid, causing its neutralization; and the pores fill with water and salt.

Were the wood left in the vat after the 70 cover is removed, the cold air entering the vat would cause the wood to soak up or absorb more and cooler water; and close the pore surface openings to a degree and encase them sufficiently to retain much of the water held in the pores, as in the present 75 and prior practices of seasoning wood.

Wherefore the immediate transfer of the wood from the vat to the kiln is a very essential feature of my invention.

By thrusting the wood from the vat into 80 the kiln heated to 250° F. instantly the pores of the wood are shrunken and closed and all the water, salt and neutralized tannic acid are squeezed out as is water from a sponge when crushed in the hand.

Thereupon the sides of the pores are brought into contact and the pores are closed and upon withdrawal of the wood at the 85 end of forty-two hours there is practically a homogeneous mass with no air, water or holes inside, and there can be no further shrinkage by reason of heat in houses or other places where the wood is subsequently used.

By my process the wood becomes one 95 hundred per cent seasoned instead of being from sixty to eighty per cent freed from water, etc., as in other known processes or when seasoned by exposure for months or years in the original way.

The temperature of the kiln (250° F.) is 100 an element of my invention because a lower heat does not close the pores quickly enough and a higher temperature burns it too much, and the length of time for its retention 105 (forty-two hours) in the kiln is essential as that much time is required to eject all moisture and close the pores and a longer ex-

posure tends to drying the wood too much, leading to a more or less powdered condition of its texture when ready for use.

For seasoning woods other than oak my invention is applied by leaving the wood in the vat with the boiling, salted water; and in the kiln, after removal thereto, a length of time respectively proportionate to the known relative proportion of tannic acid contained in each wood which is to be treated.

As stated above, therefore, I do not claim

the soaking of wood to be seasoned, in a solution of salt and water in a vat and its subsequent drying in a kiln, but I claim:—

The process of seasoning and shrinking wood consisting in boiling it six hours in an enclosed vat containing a solution of water and five per cent salt; immediate removal therefrom to a kiln heated to 250° F. and its removal from said kiln at the end of forty-two hours.

In testimony whereof I affix my signature.

ATLAS O. CRAIL.